

Patented Aug. 6, 1929.

1,723,230

# UNITED STATES PATENT OFFICE.

GEORGE HOLLAND ELLIS, OF SPONDON, NEAR DERBY, ENGLAND, ASSIGNEE TO  
CELANESE CORPORATION OF AMERICA, A CORPORATION OF DELAWARE.

## TREATMENT OF CELLULOSE ACETATE.

No Drawing. Application filed September 11, 1925, Serial No. 55,882, and in Great Britain September 23, 1924.

This invention relates to the dyeing, printing or stencilling of acetyl cellulose in yarn, thread, fabric, film or other form, and it has for its principal object to produce or render 5 dyeings or colourings thereon of improved fastness to light.

The invention may be employed in connection with any dyes, colouring matters or colouring compounds applicable for the dyeing, printing or stencilling of cellulose acetate and is of especial value in connection 10 with those of poor or relatively low resistance to light.

Among the dyestuffs or colouring matters 15 or compounds which are applicable for the dyeing, printing or stencilling of acetyl cellulose, whether already known or specially synthesized therefor, and whether soluble or insoluble in water, a number give shades on 20 acetyl cellulose which are of poor or relatively poor resistance to the fading action of light.

I have made the remarkable discovery that 25 dyeings or colourings yielded on acetyl cellulose by such dyestuffs, colouring matters or compounds can be very greatly improved in 30 resistance to light by treatment of the dyed, printed or stencilled acetyl cellulose goods (all hereinafter in the claims included in the term coloured materials comprising cellulose 35 acetate) with one or more agents being simple organic amino compounds, which term likewise includes substituted amino compounds, and that even in the case of dye- 40 stuffs, colouring matters or colouring compounds giving dyeing or colourings of good fastness to light on acetyl cellulose, the resistance to light of the shades can be improved by such after-treatment.

45 The amino compounds which I have found particularly efficacious for the purpose are aniline and substituted or alkylated anilines or alkylated phenylene diamines such as the tetra-ethyl-phenylene-diamines.

50 Among such substances I have found that the degree of efficacy increases with the degree of alkylation, thus mono-ethyl-aniline is better than aniline itself, whilst diethyl aniline is better than the mono compounds in its protective action.

55 The amino compound or compounds may be applied through any suitable media, for instance in the form of their hydrochloride or other soluble salt. Or they may be "solubilized" or "dispersed" by treatment with

solubilizing or dispersing agents of the character referred to in my prior British specification No. 219349, No. 224925 or No. 22153/1924, or in the prior British specification of the present applicant and W. O. Goldthorpe 60 No. 19292/1924, and in the U. S. applications Serial Nos. 664780, 664781, 50525, and 48666 corresponding respectively to said British specifications.

The solubilizing or dispersing agents referred to in my said British Specification 65 219349 and in my corresponding U. S. application Serial No. 664,780 are, as therein stated, bodies of oily or fatty characteristics or salts thereof, namely sulphorcinoleic acid 70 and other sulphonated fatty acids, or salts of such acids such as their alkali or ammonium salts, or other bodies having oily or fatty characteristics, i. e. higher fatty acids or sulphonated or other derivatives thereof containing 75 salt-forming groups or salts of such acids or bodies such as their alkali or ammonium salts or mixtures of any of these bodies or salts.

The solubilizing or dispersing agents referred to in the said British Specification 224925 and corresponding U. S. application Serial No. 664,781 are carbocyclic compounds containing in their structure one or more salt-forming groups (whether the compound 80 contains only one kind of these groups or different kinds of these groups at the same time) or sodium or other salts of said compounds, and may be used alone or in mixture with the solubilizing or dispersing 85 agents of the said British Specification 219349 and corresponding U. S. application Serial No. 664,780. They comprise a wide range of organic derivatives containing in their structure one or more salt-forming 90 groups such as the sulphonic, carboxyl or hydroxyl groups, whether the compound contains only one kind or different kinds of these groups; for example said carbocyclic 95 compounds comprise phenols, sulphonic acids, carboxylic acids, phenol sulphonic acids or other derivatives of the benzene, naphthalene or anthracene series, containing one or more of any of the said groups; or derivatives of other cyclic hydrocarbons, saturated or non- 100 saturated, containing one or more of the above mentioned groups, such for example as the naphthenic acids (such as occur naturally in Caucasian petroleum), naphthene sulphonic acids or other carboxylic or sul-

105 110

phonic acids of the cycloparaffins; or the sodium or other salts of any of the derivatives referred to.

The solubilizing or dispersing agents referred to in the said British Specification No. 22153/1924 and corresponding U. S. application Serial No. 50,525 comprise sulpho aromatic acids such as sulpho benzene stearic acid (Twitchell reagent), or derivatives thereof, such as sulpho phenol stearic acid or sulpho naphthalene stearic acid, or salts of such bodies.

In the said British specification of the present applicant and W. O. Goldthorpe, No. 19292/1924 and corresponding U. S. application Serial No. 48,666, bodies therein termed secondary or auxiliary solvents are employed in conjunction with sulphoricinoleic acid or other bodies of oily or fatty 20 characteristics such as hereinbefore referred to, or with salts of such bodies. As stated in the said specification, such secondary or auxiliary solvents comprise a wide range of chemical compounds, and those found especially useful comprise alkyl or alkylene halides, such for instance as tetrachlorethane, trichlorethylene; simple or "mixed" derivatives of the cyclic or aromatic series containing one or more amino, chlor, or 30 hydroxy groups, such for example as cresols, alkylanilines, toluidines, chlorphenols, mono or polychlor benzenes; hydrogenated derivatives of such or other aromatic compounds, such for example as hexahydrophenol, hexahydrocresols, hexadrobenzene, dekahydronaphthalene, tetrahydronaphthalene and the like.

Where the amino compound itself has a sufficient water solubility it can of course be applied as such in plain aqueous solution. Some of such simple amino compounds show the tendency themselves to undergo oxidation on exposure under the catalytic influence of light, giving dark coloured products, for 40 example diphenylamine, para-amidophenol, paraphenylene diamine. Thus we prefer to use those such as are first instanced above and which do not show this property to an appreciable degree.

Colouring matters, the shades of which on acetyl cellulose are greatly enhanced in resistance to light by the above methods fall within many different classes, but the improvement has been found more generally marked in the "azo" class. Examples of some colouring matters yielding shades loose to light in the ordinary way but enormously improved by treatments according to the invention are: benzeneazoalphanaphthylamine, benzeneazophenylmethylpyrazolone, benzeneazobenzeneazobetanaphthol, quinophthalone (quinoline yellow base), alpha-amidoazonaphthalene.

A very great advantage of the processes of the present invention is that such simple

organic amino compounds referred to are absorbed readily from aqueous solutions or dispersions by the acetyl cellulose in its various forms, so that the quantities required are relatively small and the strengths of the solutions relatively low as compared with what would be necessary in applying an agent merely mechanically.

The following is an example illustrating how the invention may be carried out, it being understood that this is given simply by way of example and can be varied widely.

*Example.*

100 lbs. of acetyl cellulose knitted fabric is dyed in any suitable manner with an aqueous hydrochloric acid solution of benzene-azoalphanaphthylamine. The fastness to light of the yellow shade thus achieved is very poor. Three pounds of diethylaniline hydrochloride are now dissolved in water and added to a fresh aqueous bath and the above dyed material worked in this until no more amine is absorbed. The shade now obtained will be of very much superior resistance to the action of light.

The invention may of course be applied to dyed, printed or stencilled goods whether consisting wholly of cellulose acetate filaments or fibres or consisting partly thereof and partly of another or other fibre or fibres, as for example in mixed yarns or fabrics, and all such goods are referred to in the claims as colored materials comprising cellulose acetate.

What I claim and desire to secure by Letters Patent is:—

1. Process for the treatment of colored materials comprising cellulose acetate for the purpose of increasing their fastness to light, said process comprising treating said materials with at least one simple organic amino compound.

2. Process for the treatment of colored materials comprising cellulose acetate for the purpose of increasing their fastness to light, said process comprising treating said materials with at least one simple organic amino compound in the form of its hydrochloride.

3. Process for the treatment of colored materials comprising cellulose acetate for the purpose of increasing their fastness to light, said process comprising treating said materials with a simple aromatic amino compound.

4. Process for the treatment of colored materials comprising cellulose acetate for the purpose of increasing their fastness to light, said process comprising treating said materials with a simple alkylated aniline.

5. Process for the treatment of colored materials comprising cellulose acetate for the purpose of increasing their fastness to light, said process comprising treating said

materials with an alkylated aniline in the form of its hydrochloride.

6. Process for the treatment of colored materials comprising cellulose acetate for the purpose of increasing their fastness to light, said process comprising treating said materials with diethylaniline.

7. Process for the treatment of colored materials comprising cellulose acetate for the purpose of increasing their fastness to light, said process comprising treating said

materials with diethylaniline in the form of its hydrochloride.

8. Process for the treatment of colored materials comprising cellulose acetate for the purpose of increasing their fastness to light, said process comprising treating said materials with a simple aromatic amino compound in the form of its hydrochloride.

In testimony whereof I have hereunto subscribed my name.

GEORGE HOLLAND ELLIS.